

# UNITED STATES PATENT OFFICE.

WILLIAM G. LINDSAY, OF NEWARK, NEW JERSEY, ASSIGNOR TO THE CELLULOID COMPANY, A CORPORATION OF NEW JERSEY.

## ACETYL-CELLULOSE PROCESS AND PRODUCT.

1,236,579.

Specification of Letters Patent. Patented Aug. 14, 1917.

No Drawing.

Application filed July 11, 1914. Serial No. 850,432.

*To all whom it may concern:*

Be it known that I, WILLIAM G. LINDSAY, a citizen of the United States, residing at Newark, in the county of Essex and State 5 of New Jersey, have invented certain new and useful Improvements in Acetyl-Cellulose Processes and Products, of which the following is a full, clear, and exact specification.

10 This invention relates to acetyl-cellulose and a process of making the same. Its object is to accomplish acetylation of the cellulose in fibrous form, without solution of the cellulose, and without the use of sulfuric 15 acid, sulfo-acids, or other constituents tending to induce decomposition.

In practice I proceed as follows:

Cellulose, preferably high grade bleached cotton rovings, is given a preliminary treatment 20 with acetic acid and zinc chlorid. For best results the cellulose should contain a normal amount of moisture, generally from 2% to 4%. I prefer about 3½%. The acetic acid should be about 90% strength, 25 and the zinc chlorid should be pure, free from iron and substantially anhydrous. A good example of proportions is cellulose 100 parts, acetic acid 200 parts and zinc chlorid 50 parts. The zinc chlorid is dissolved 30 in the acetic acid at ordinary room temperature by agitation and the solution thus produced is poured on to the cellulose contained in a suitable stoneware receptacle and allowed to penetrate. The position of 35 the cellulose is changed from time to time and the reaction is allowed to proceed for forty-eight hours at a room temperature of from 60° to 70° F.

After the foregoing preliminary treatment, 40 the impregnated cellulose is subjected to the acetylating bath, which consists of acetic anhydrid and benzene. For best results the acetic anhydrid should be of the highest commercial purity obtainable— 45 about 92½%. The benzene is of the so-called commercial chemically pure variety. A good example of proportions, consistent with the forgoing proportions for preliminary treatment, is acetic anhydrid 450 parts, 50 benzene 1650 parts. The acetic anhydrid and benzene are mixed and the mixture warmed in a suitable vessel, such as an enameled steel kettle, to a temperature of about 150° F. The preliminarily treated

cellulose is introduced into this mixture, 55 the temperature being controlled by means of a water or air bath, adjusted at 150° F. Due to the reaction the temperature of the mixture rises rapidly at the start, reaching about 165° F. in about ten minutes, then 60 rises more slowly to about 170° F. in about an hour, and then slowly and gradually drops until the temperature of the water bath (150° F.) is reached. This ordinarily 65 takes place in about twelve hours. When this temperature has been reached the product may be removed from the bath, or the reaction may be continued, depending upon the nature of the product desired. In many cases the product resulting from the reaction 70 of twenty-four hours is desirable.

In the preliminary treatment, the bath of acetic acid, water and zinc chlorid may be composed of any suitable equivalents for its ingredients, for example the water may 75 be substituted by any other suitable hydroxyl containing substance which, like water, is neutral with respect to the cellulose and miscible with the acetylizing bath but will act to induce acetylation; in place 80 of acetic acid other suitable diluent may be employed, and in place of zinc chlorid as a condensing agent other suitable inorganic salts may be employed.

At the end of the reaction period the 85 product is freed from the spent acetylating liquor by any suitable means; for example, by whizzing or by pressing. After the bulk of the spent acetylating liquor has been separated from the acetyl-cellulose, the 90 balance is then removed by washing the acetyl-cellulose in hot water, or, if preferred, by means of a suitable vacuum machine.

The product thus obtained exhibits a physical form identical with the raw cotton, and is soluble in acetylene tetrachlorid, 95 and with difficulty in chloroform.

Having thus described my invention, I declare that what I claim as new and desire to secure by Letters Patent is:—

100 1. The process of acetylizing cellulose which consists in treating cellulose with a preliminary bath of zinc chlorid, acetic acid and water, and then subjecting the impregnated cellulose to the action of an acetylating bath.

105 2. The process of acetylizing cellulose which consists in treating cellulose with a

preliminary bath of zinc chlorid, acetic acid and water, and then subjecting the impregnated cellulose to the action of a non-solvent acetylizing bath.

5. 3. The process of acetylizing cellulose which consists in treating cellulose with a preliminary bath of a non-acid condensing agent, acetic acid and water, and then subjecting the impregnated cellulose to the action of a non-solvent acetylizing bath.

10. 4. The process of acetylizing cellulose which consists in treating cellulose with a preliminary bath which comprises a non-acid condensing agent and is miscible with 15 the acetylizing bath and which does not alter the cellulose as such and acts to induce later acetylation, and then subjecting the treated cellulose to the action of a non-solvent acetylating bath containing no additional condensing agent.

15. 5. The process of acetylizing cellulose which consists in treating cellulose with a preliminary bath containing zinc chlorid and an agent which acts to induce acetylation without altering the cellulose as such and is miscible with the acetylizing bath, and then subjecting the impregnated cellulose to the action of a non-solvent acetylating bath.

20. 6. The process of acetylizing cellulose which consists in treating approximately 100 parts of cellulose with 200 parts of 90% acetic acid and 50 parts of zinc chlorid, and subjecting the impregnated cellulose to the action of a non-solvent acetylizing bath.

25. 7. The process of acetylizing cellulose which consists in treating approximately 100 parts of cellulose with 200 parts of 90% acetic acid and 50 parts of zinc chlorid, and subjecting the impregnated cellulose to an acetylating bath of 450 parts acetic anhydrid and 1650 parts benzene.

30. 8. The process of acetylizing cellulose which consists in treating cellulose with a 45 hydroxyl containing substance which acts to induce acetylation without altering the cellulose as such and is miscible with the acetylizing bath, a diluent therefor and a non-acid condensing agent, and then subjecting the impregnated cellulose to the action of a non-solvent acetylating bath.

35. 9. The process of acetylizing cellulose which consists in treating cellulose with a hydroxyl-containing substance which acts to induce acetylation without altering the cellulose as such and is miscible with the acetylizing bath, a diluent therefor and a condensing agent consisting of an inorganic salt, and then subjecting the impregnated cellulose to the action of a non-solvent acetylating bath.

40. 10. The process of acetylizing cellulose which consists in treating cellulose with a hydroxyl containing substance which acts 65 to induce acetylation without altering the

cellulose as such and is miscible with the acetylizing bath, a diluent therefor and a non-acid condensing agent, and then subjecting the impregnated cellulose to the action of an acetylating bath of acetic anhydrid and benzene.

45. 11. The process of acetylizing cellulose, which consists in first impregnating the cellulose with a preliminary bath comprising a condensing agent and an ingredient 75 that will facilitate later acetylation and then subjecting the treated cellulose to a second bath comprising an acetylating agent without any additional condensing agent.

50. 12. The process which consists in treating cellulose with zinc chlorid and a diluent which does not react with the cellulose, and then subjecting the treated cellulose to an acetylating bath.

55. 13. The process which consists in treating cellulose with zinc chlorid and hydrous acetic acid, and then subjecting the treated cellulose to an acetylating bath.

60. 14. The process which consists in treating cellulose with zinc chlorid and a diluent 90 which does not react with the cellulose, and then subjecting the treated cellulose to a reactive bath of an acetylating agent and a diluent of said agent in which the cellulose is insoluble.

65. 15. The process which consists in treating cellulose with zinc chlorid and a diluent which does not react with the cellulose, and then subjecting the treated cellulose to a reactive bath of acetic anhydrid and benzene.

70. 16. The process which consists in treating cellulose with a non-acid condensing agent and a hydroxyl containing substance which acts to induce acetylation without altering 105 the cellulose as such and is miscible with the acetylizing bath, both of which are diluted with a diluent which does not react upon the cellulose, and then subjecting the treated cellulose to an acetylating bath.

75. 17. The process which consists in treating cellulose with a non-acid condensing agent and a hydroxyl containing substance which acts to induce acetylation without altering the cellulose as such and is miscible with the acetylizing bath, both of which are diluted with a diluent which does not react upon the cellulose, and then subjecting the treated cellulose to a reactive bath containing an acetylating agent and a diluent of said agent in which the cellulose is insoluble.

80. 18. The process which comprises treating cellulose first with a non-acid condensing agent and thereafter with an acetylizing agent and a diluent of said acetylizing agent 125 in which the cellulose is insoluble.

85. 19. The process which comprises treating cellulose with an inorganic salt which acts as a condensing agent and then with an acetylizing agent, and a diluent of said 130

acetylizing agent in which the cellulose is insoluble.

20. The process of acetylizing cellulose, which comprises treating the cellulose, and with zinc chlorid, and thereafter with an acetylizing agent and a diluent of said acetylizing agent in which the cellulose is insoluble.

21. The process of acetylizing cellulose which comprises treating the cellulose with zinc chlorid and thereafter with an acetylizing agent and benzene.

22. The process of acetylizing cellulose which cónsists in treating cellulose with a hydroxyl containing substance which acts to induce acetylation without altering the cellulose as such, and is miscible with the acetylizing bath, a diluent therefor and a non-acid condensing agent, and then subjecting the same to the action of an acetylizing bath of acetic anhydrid and a diluent therefor in which the cellulose is insoluble.

23. The product which comprises acetyl cellulose obtained by treating cellulose with a non-acid condensing agent and a hydroxyl containing substance which acts to induce acetylation without altering the cellulose as such and is miscible with the acetylizing bath, both of which are diluted with a diluent which does not react upon the cellulose, and then subjecting the treated cellulose to an acetylizing bath.

24. The product which comprises acetyl cellulose obtained by treating cellulose with a non-acid condensing agent and a hydroxyl containing substance which acts to induce acetylation without altering the cellulose as such and is miscible with the acetylizing bath, both of which are diluted with a diluent which does not react upon the cellulose, and then subjecting the treated cellulose to a reactive bath of an acetylizing agent and a

diluent of said agent in which the cellulose is insoluble.

25. The product which comprises acetyl cellulose obtained by treating cellulose with a non-acid condensing agent and a hydroxyl containing substance which acts to induce acetylation without altering the cellulose as such and is miscible with the acetylizing bath, both of which are diluted with a diluent which does not react upon the cellulose, and then subjecting the treated cellulose to a reactive bath of acetic anhydrid and benzene.

26. A product of the hereinbefore described process comprising an acetyl cellulose, the original fibrous structure of the cellulose being substantially unaltered, the product being obtained without hydrolysis of the cellulose and being difficultly but nevertheless soluble in chloroform.

27. The product which comprises acetyl cellulose obtained without hydrolysis of the cellulose by treating it with a condensing agent and a substance that acts to facilitate later acetylation and then with an acetylizing bath.

28. The product which comprises acetyl cellulose obtained by treating cellulose with a non-acid condensing agent and a substance which acts to facilitate later acetylation and is miscible with the later acetylizing bath and which does not perceptibly alter the chemical composition of the cellulose and thereafter subjecting the treated cellulose to an acetylizing bath.

In testimony whereof I affix my signature, in presence of two witnesses.

WILLIAM G. LINDSAY.

Witnesses:

C. V. EDWARDS,  
C. GALVION.